

# United States Patent [19]

Shimizu et al.

[11] Patent Number: 4,508,790

[45] Date of Patent: Apr. 2, 1985

[54] TIN FREE STEEL HAVING AN EXCELLENT WELDABILITY AND ITS PRODUCTION METHOD

[75] Inventors: Nobuyoshi Shimizu; Terunori Fujimoto; Tsuneo Inui; Masatoki Ishida, all of Yamaguchi, Japan

[73] Assignee: Toyo Kohan Co., Ltd., Tokyo, Japan

[21] Appl. No.: 619,271

[22] Filed: Jun. 11, 1984

[51] Int. Cl.<sup>3</sup> ..... C25D 5/12; C25D 5/34; C25D 5/48; C25D 11/38

[52] U.S. Cl. ..... 428/632; 204/29; 204/35.1; 204/41; 204/44.2; 204/44.5; 204/129.75; 428/658; 428/666; 428/680

[58] Field of Search ..... 204/41, 29, 35.1; 428/632, 666, 680, 658; 427/328, 383.7, 405

[56] References Cited

U.S. PATENT DOCUMENTS

4,064,320 12/1977 Adaniya et al. ..... 428/632  
4,157,944 6/1979 Inui et al. ..... 204/41  
4,414,078 11/1983 Shimizu et al. ..... 204/34  
4,432,842 2/1984 Inui et al. ..... 204/41

Primary Examiner—G. L. Kaplan

Attorney, Agent, or Firm—Wenderoth, Lind & Ponack

[57]

## ABSTRACT

Tin free steel having three layers consisting of a bottom layer of metallic chromium, a middle layer of nickel-zinc alloy containing 10 to 90 weight percent of zinc and a top layer of hydrated chromium oxide on a steel base, and a method for the continuous production of this tin free steel which comprises:

(a) chromium plating a steel base to form a layer of metallic chromium and hydrated chromium oxide, (b) nickel-zinc alloy plating the chromium plated steel base by using a nickel-zinc alloy plating electrolyte sufficiently acidic to dissolve the hydrated chromium oxide and (c) forming a hydrated chromium oxide layer on the chromium plated nickel-zinc plated steel base.

Instead of (b) in the above method, a cathodic treatment in an acidic solution can be carried out for the removal of hydrated chromium oxide formed during chromium plating, and thereafter nickel-zinc alloy plating can be carried out by using a known nickel-zinc alloy plating electrolyte.

This tin free steel is useful for producing welded can bodies at high speed without removing the plated layer in the welded part, since it has an excellent weldability.

19 Claims, No Drawings

**TIN FREE STEEL HAVING AN EXCELLENT  
WELDABILITY AND ITS PRODUCTION METHOD**

**FIELD OF THE INVENTION**

The present invention relates to a tin free steel having an excellent weldability, excellent lacquer adhesion and excellent sulfite stain resistance and method for its production. In detail, the invention relates to a tin free steel having three layers consisting of a bottom layer (layer closest to the steel base) of metallic chromium, a middle layer of nickel-zinc alloy and a top layer (layer farthest from the steel base) of hydrated chromium oxide on a steel base, and a method for production of this tin free steel which is characterized by nickel-zinc alloy plating after chromium plating by using a nickel-zinc alloy plating electrolyte having a pH of 0.5 to 2.0 or by nickel-zinc alloy plating by using a known nickel-zinc alloy plating electrolyte after a removal of a hydrated chromium oxide formed during chromium plating by using an acidic solution having a pH of 0.5 to 2.0.

This tin free steel is useful for producing welded can bodies at high speed without removing the plated layer in the welded part.

**BACKGROUND AND OBJECTIVE**

Recently the change from expensive electrotinplates to cheaper tin free steel (TFS-CT) having double layers consisting of a lower layer of metallic chromium and an upper layer of hydrated chromium oxide as well as a decrease in the weight of the tin coating in electrotinplates has rapidly taken place in the field of food cans.

This is because the tin used for the production of tinplate is very expensive and there is concern over the exhaustion of tin resources in the world.

An ordinary metal can consists of two can ends and a single can body, except for drawn cans. In the case of tinplate, the seaming of the can body is generally carried out by soldering. In this soldering process, however, it is impossible to decrease the weight of the tin coating on the tinplate to under 2.8 g/m<sup>2</sup>, because it is difficult to stabilize the soldering process when the weight of the tin coating is under 2.8 g/m<sup>2</sup>. From the regulation of lead content in the solder used for the seaming of the tinplate can body in the field of food cans, the seaming of the tinplate can body is widely carried out by electric welding. A lap seam welding, for instance, the Soudronic process, has been recently used for the seaming of the tinplate can body.

In this process, it is desirable to decrease the tin coating weight in the tinplate, but the weldability of tinplate becomes poor with a decrease of the tin coating weight.

On the other hand, the seaming of a TFS-CT can body is generally carried out with nylon adhesives using Toyo Seam (trademark) and Mira Seam (trademark) methods. Another method of seaming a TFS-CT can body by electric welding is also well known. In the case of the seaming of a TFS-CT can body by electric welding, however, the metallic chromium layer and the hydrated chromium oxide layer must be mechanically removed from the TFS-CT surface in order to easily weld the TFS-CT can body at high speed. Therefore, the corrosion resistance in the welded part of the TFS-CT can body becomes remarkably poor, even if this welded part is coated with lacquer after welding.

From the background described above, the development of a can material which is cheaper than tinplate, is

easily welded at high speed without the removal of the plated layer, has been required in the field of food cans.

Recently, various surface treated steel sheets have been proposed as a can material which can be easily welded at high speed without the removal of the plated layer. For instance, the following surface treated steel sheets have been proposed:

- (a) Lightly tin coated steel sheet (LTS) with below about 1.0 g/m<sup>2</sup> of tin which is reflowed or unreflowed after tin plating (Japanese Patent Publication Nos. Sho 56-3440, Sho 56-54070, Sho 57-55800, and Laid-Open Japanese Patent Application Nos. Sho 56-75589, Sho 56-130487, Sho 56-156788, Sho 57-101694, Sho 57-185997, Sho 57-192294, Sho 57-192295 and Sho 55-69297).
- (b) Nickel preplated LTS with below about 1.0 g/m<sup>2</sup> of tin (Laid-Open Japanese Application Nos. Sho 57-23091, Sho 57-67196, Sho 57-110685, Sho 57-177991, Sho 57-200592 and Sho 57-203797).
- (c) Nickel plated steel sheet with chromate film or phosphate film (Laid-open Japanese Patent Application Nos. Sho 56-116885, Sho 56-169788, Sho 57-2892, Sho 57-2895, Sho 57-2896, Sho 57-2897, Sho 57-35697 and Sho 57-35698).
- (d) TFS-CT having double layers consisting of a lower layer of metallic chromium and an upper layer of hydrated chromium oxide which is obtained by some special methods such as cold rolling after TFS treatment (Laid-open Japanese Patent application No. Sho 55-48406), porous chromium plating (Laid-open Japanese Patent Application No. Sho 55-31124) and a cathodic treatment of a steel sheet in chromic acid electrolyte with fluoride but without anions such as sulfate, nitrate and chloride ions (Laid-open Japanese Patent Application No. Sho 55-18542).

However, LTS and nickel preplated LTS above identified as (a) and (b) are slightly more expensive than TFS-CT. Furthermore, these have not only narrower available current range for sound welding than that in tinplate, but also poor lacquer adhesion compared with that in TFS-CT, although these can be welded without the removal of the plated layer. The reason why the available current range for sound welding in LTS and nickel preplated LTS is narrower than in tinplate is considered to be that the amount of free tin in these is smaller than that in tinplate and also further decreases because of changes of free tin to iron-tin alloy by heating for lacquer curing. Nickel plated steel sheet with chromate film or phosphate film identified above as (c) also has narrower available current range for sound welding than that in LTS or nickel preplated LTS. Furthermore, the corrosion resistance of nickel plated steel sheet is poorer than that in TFS-CT, although the lacquer adhesion of nickel plated steel sheet is good.

Particularly, pitting corrosion in the defective part of the lacquered nickel plated steel sheet may occur easily from acidic foods such as tomato juice because the electrochemical potential of nickel is more noble than that of steel base and metallic chromium.

It is considered that the welding of TFS-CT identified above as (d) without the removal of TFS-CT film at high speed is very difficult because the oxide films having high electric resistance are formed by the oxidation of metallic chromium and exposed steel base and by the dehydration of hydrated chromium oxide during heating for curing the lacquer coating on the TFS-CT can

body, although TFS-CT identified above as (d) may be welded when it is not heated before welding.

As described above, various surface treated steel sheets proposed in (a), (b), (c) and (d) have various problems in the production cost and the characteristics as a can material which can be easily welded without the removal of the plated layer at high speed.

Accordingly, it is the first objective of the present invention to provide a tin free steel sheet having an excellent weldability, that is, easily being welded without the removal of the plated layer at high speed, and having excellent corrosion resistance after lacquering such as that in TFS-CT.

It is the second objective of the present invention to provide a method for the continuous production of a tin free steel having an excellent weldability.

#### BRIEF DESCRIPTION OF THE INVENTION

The first objective of the present invention can be accomplished by providing a tin free steel (TFS-20 CNZT) having three layers consisting of a bottom layer of metallic chromium, a middle layer of nickel-zinc alloy and a top layer of hydrated chromium oxide on a steel base.

The second objective of the present invention can be 25 accomplished by a nickel-zinc alloy plating on the chromium plated steel base. More specifically, the method of the present invention is characterized by a nickel-zinc alloy plating onto the chromium plated steel base wherein nickel-zinc alloy is carried out at the same time with the removal of hydrated chromium oxide formed during chromium plating by using a nickel-zinc alloy plating electrolyte having a low pH such as 0.5 to 2.0 which has a low current efficiency for nickel-zinc alloy plating. Another method of the present invention is 35 characterized by a nickel-zinc alloy plating onto the chromium plated steel base by using a known nickel-zinc alloy plating electrolyte after the removal of hydrated chromium oxide forming during chromium plating by a cathodic treatment of the chromium plated 40 steel base in an acidic solution having a pH of 0.5 to 2.0.

The TFS-CNZT according to the present invention can be used in applications wherein excellent weldability, that is, easily being welded without the removal of the plated layer at high speed, is required such as food can bodies, aerosol can bodies and miscellaneous can bodies which are lacquered except for the welded part before welding.

The TFS-CNZT according to the present invention can be also used in applications wherein the lacquer coating is not carried out because it has an excellent weldability. Furthermore TFS-CNZT can be used in applications wherein excellent corrosion resistance after lacquering are required, such as can ends, drawn cans and drawn and redrawn cans (DRD cans), besides can bodies.

#### DETAILED DESCRIPTION OF THE INVENTION

The steel base used for the production of the TFS-CNZT according to the present invention can be any cold rolled steel sheet customarily used in manufacturing electrotinplate and TFS-CT. Preferably, a type of steel base for electrotinplate, as set out in ASTM A 623-76 of 1977 (standard specification for general requirements for tin mill product), is employed as the steel base. Preferably, the thickness of the steel base is from about 0.1 to about 0.35 mm.

The TFS-CNZT according to the present invention is produced by the following processes: (1) degreasing with an alkali and pickling with an acid→water rinsing→chromium plating→water rinsing→nickel-zinc alloy plating with the removal of hydrated chromium oxide→water rinsing→chromate treatment→water rinsing→drying or (2) degreasing with an alkali and pickling with an acid→water rinsing→chromium plating→water rinsing→the removal of hydrated chromium oxide by a cathodic treatment in an acid solution→water rinsing→nickel-zinc alloy plating→water rinsing→chromate treatment→water rinsing→drying.

By using these processes identified above as (1) and (2), three layers consisting of a bottom layer of metallic chromium, a middle layer of nickel-zinc alloy and a top layer of hydrated chromium oxide are formed on a steel base. In the present invention, the amount of each layer is very important in order to obtain an excellent weldability which is an objective of the present invention, besides the conditions in each process.

At first, the amount of metallic chromium being a bottom layer in the TFS-CNZT according to the present invention should be controlled to the range of 30 to 300 mg/m<sup>2</sup>, more preferably 70 to 150 mg/m<sup>2</sup>. If the amount of metallic chromium is below 30 mg/m<sup>2</sup>, the excellent weldability and the excellent corrosion resistance are not obtained because the surface of a steel base is not sufficiently covered with the plated metallic chromium. The amount of metallic chromium is limited to 300 mg/m<sup>2</sup> from an economical and an industrial point of view.

Secondly, the amount of nickel-zinc alloy being a middle layer in the TFS-CNZT according to the present invention should be controlled to the range of 5 to 300 mg/m<sup>2</sup>, more preferably 10 to 50 mg/m<sup>2</sup>. If the amount of nickel-zinc alloy plated on the chromium plated steel base is below 5 mg/m<sup>2</sup>, the excellent weldability is not obtained, because chromium oxide, having high electrical resistance, is formed by the oxidation of metallic chromium during heating for lacquer curing, even if the oxidation of a steel base is prevented by the sufficient amount of metallic chromium. The amount of the plated nickel-zinc alloy is limited to 300 mg/m<sup>2</sup> from an industrial point of view, although the affect of nickel-zinc alloy in the present invention does not change in an amount above 300 g/m<sup>2</sup>.

In the present invention, nickel-zinc alloy does not mean a nickel-zinc alloy having a stoichiometrical composition with a constant ratio of zinc to nickel, but means the co-deposition of zinc and nickel having various ratios of zinc to nickel. In the present invention, zinc content or nickel content in the plated nickel-zinc alloy is very important in order to obtain the excellent characteristics in the weldability, sulfide stain resistance and lacquer adhesion.

The weldability is gradually improved with an increase of zinc content in the plated nickel-zinc alloy, because the electric contact resistance of the TFS-CNZT is decreased with an increase of zinc which has a low melting point compared with that of nickel.

Furthermore, the sulfide stain resistance is also gradually improved with an increase of zinc content in the plated nickel-zinc alloy, because white zinc sulfide is formed by the preferential reaction of zinc with sulfide ion produced from protein containing foods such as fish and meat during the retort treatment without forming a black nickel sulfide.

However, the lacquer adhesion becomes gradually poor with an increase of zinc content in the plated nickel-zinc alloy. Therefore, the zinc content in the plated nickel-zinc alloy should be controlled in the range of 10 to 90 weight percent, more preferably 10 to 50 weight percent to the total weight of the plated nickel and zinc, because the affects of co-deposited zinc described above are not observed at below 10 weight percent or above 90 weight percent of zinc in the plated nickel-zinc alloy. Particularly, it is difficult to stably plate nickel-zinc alloy having below 10 weight percent of zinc on the chromium plated steel base, because it is necessary to exactly control the concentration of zinc ion in the nickel-zinc alloy plating electrolyte in below 0.5 g/l of zinc ion.

Zinc plating after nickel plating and nickel plating after zinc plating on the chromium plated steel base are considered in order to obtain the TFS-CNZT having excellent characteristics in weldability, sulfide stain resistance and lacquer adhesion, but these methods are not suitable for the production of the TFS-CNZT because a complex process is required.

As described above, the presence of metallic chromium as a bottom layer and nickel-zinc alloy as a middle layer in the TFS-CNZT according to the present invention are indispensable in order to obtain excellent characteristics in weldability, sulfide stain resistance and lacquer adhesion.

Furthermore in the present invention, the presence of a small amount of hydrated chromium oxide as a top layer is indispensable in order to prevent the oxidation of the exposed steel base and the exposed metallic chromium after nickel-zinc alloy plating during heating for lacquer curing and to obtain the excellent corrosion resistance and the excellent lacquer adhesion.

The optimum range in the amount of hydrated chromium oxide is from 2 to 18 mg/m<sup>2</sup>, more preferably 4 to 12 mg/m<sup>2</sup> as chromium.

If the amount of hydrated chromium oxide is below 2 mg/m<sup>2</sup> as chromium, the corrosion resistance and the lacquer adhesion become poor. If the amount of hydrated chromium oxide is above 18 mg/m<sup>2</sup>, the weldability becomes remarkably poor because hydrated chromium oxide changes to chromium oxide having high electric resistance by dehydration during heating for lacquer curing.

The conditions for each process in the production of the TFS-CNZT according to the present invention are shown in detail.

At first, in order to form a metallic chromium layer as a bottom layer of the TFS-CNZT according to the present invention, a known chromium plating electrolyte such as a Sargent bath or a chromic acid electrolyte containing additives such as fluorine compounds and sulfur compounds which are used for the production of TFS-CT having a lower layer of metallic chromium and an upper layer of hydrated chromium oxide, may be employed.

In the present invention, it is preferable to employ the following electrolytic chromium plating conditions for the formation of a metallic chromium layer on a steel base:

Concentration of chromic acid: 30-300 g/l, more preferably 80-300 g/l

Concentration of additives: 1.0-5.0 weight %, more preferably 1.0-3.0 weight % of the concentration of chromic acid

Additives: at least one compound selected from the group consisting of fluorine compounds and sulfur compounds

Temperature of the electrolyte: 30°-60° C.

Cathodic current density: 10-100 A/dm<sup>2</sup>

Generally, the amount of hydrated chromium oxide formed during chromium plating decreases with an increase in the concentration of chromic acid in the suitable weight ratio of additives to chromic acid. It is not preferable to use an electrolyte having below 30 g/l of chromic acid for the chromium plating because the current efficiency for the deposition of metallic chromium decreases remarkably. The concentration of chromic acid above 300 g/l is not also suitable from an economical point of view.

The presence of additives such as fluorine compounds and sulfur compounds in the chromium plating electrolyte is indispensable for a uniform chromium deposition. If the weight percent of additives to chromic acid is below 1.0 or above 5.0, the current efficiency for the deposition of metallic chromium remarkably decreases, besides a decrease in uniformity of the deposited metallic chromium layer is observed.

Particularly, at below a 1.0 value for the weight percent of additives to chromic acid, the formed insoluble hydrated chromium oxide remarkably prevents the formation of a uniform nickel-zinc alloy layer in the following nickel-zinc alloy plating.

It is preferable that the additive is at least one compound selected from the group consisting of fluorine compounds such as hydrofluoric acid, fluoboric acid, fluosilicic acid, ammonium bifluoride, an alkali metal bifluoride, ammonium fluoride, an alkali metal fluoride, ammonium fluoborate, an alkali metal fluoborate, ammonium fluosilicate, an alkali metal fluosilicate, aluminum fluoride and sulfur compounds such as sulfuric acid, ammonium sulfate, an alkali metal sulfate, chromium sulfate, aluminum sulfate, phenolsulfonic acid, ammonium phenolsulfonate, an alkali metal phenolsulfonate, phenoldisulfonic acid, ammonium phenoldisulfonate, an alkali metal phenoldisulfonate, ammonium sulfite, an alkali metal sulfite, ammonium thiosulfate and an alkali metal thiosulfate.

The amount of hydrated chromium oxide formed during chromium plating decreases with an increase in the temperature of the electrolyte. The temperature of the electrolyte above 60° C. is not suitable from an industrial point of view, because the current efficiency for the deposition of metallic chromium decreases remarkably. The temperature of the electrolyte below 30° C. is not also suitable because a long time is necessary for the removal of the large amount of hydrated chromium oxide formed during chromium plating.

With an increase in cathodic current density, the current efficiency for the deposition of metallic chromium increases and the amount of hydrated chromium oxide formed during chromium plating decreases. It is suitable in the present invention that the range of the cathodic current density for the deposition of metallic chromium be 10 to 100 A/dm<sup>2</sup>, more preferably 40 to 80 A/dm<sup>2</sup>, because metallic chromium almost does not deposit at below 10 A/dm<sup>2</sup> of the current density and the current efficiency for the deposition of metallic chromium almost does not increase at above 100 A/dm<sup>2</sup> of the current density.

In the present invention, the conditions for chromium plating wherein a good current efficiency for the deposition of metallic chromium is obtained and a small

amount of hydrated chromium oxide is formed, should be selected because the presence of hydrated chromium oxide prevents the formation of a uniform nickel-zinc alloy layer in the following nickel-zinc alloy plating.

However, hydrated chromium oxide is always formed on a deposited metallic chromium layer during chromium plating.

Under the conditions of higher concentration of chromic acid, higher current density and higher temperature of the electrolyte, the amount of hydrated chromium oxide formed on the deposited metallic chromium is about 3 to 10 mg/m<sup>2</sup> as chromium. On the contrary, under the conditions of lower concentration of chromic acid, lower current density and lower temperature of the electrolyte, it is about 10 to 50 mg/m<sup>2</sup> as chromium.

When a large amount of hydrated chromium oxide is formed during chromium plating, it is possible to decrease it by leaving the chromium plated steel base in the chromium plating electrolyte for a few seconds. However, hydrated chromium oxide of about 3 to 5 mg/m<sup>2</sup> as chromium remains on the surface of the chromium plated steel base, even if the chromium plated steel base covered with hydrated chromium oxide is left in the chromium plating electrolyte for a long time.

In the present invention, this hydrated chromium oxide must be removed before the following nickel-zinc alloy plating because the presence of hydrated chromium oxide prevents the deposition of a uniform nickel-zinc alloy layer on a metallic chromium layer.

The following methods have been considered for the removal of hydrated chromium oxide on the deposited metallic chromium layer.

(A) An immersion of the chromium plated steel base before drying into a high concentration of an alkaline such as an alkali metal hydroxide and an alkali metal carbonate at high temperature of 70° to 90° C. It is difficult to industrialize this method because the alkaline solution may be mixed into the following nickel-zinc alloy plating electrolyte.

(B) An immersion of the chromium plated steel base before drying into an acid solution such as sulfuric acid and hydrochloric acid. The method is not suitable in the present invention, because the hydrated chromium oxide formed during chromium plating is not sufficiently dissolved by immersion into an acid solution for a short time.

(C) A mechanical removal of hydrated chromium oxide by a brushing roll or wiper in an alkaline solution or an acid solution before drying of the chromium plated steel base. The hydrated chromium oxide formed on the deposited metallic chromium layer is not uniformly removed by this method.

Therefore these methods such as (A), (B) and (C) are not suitable for the removal of hydrated chromium oxide before the following nickel-zinc alloy plating.

In the present invention, the following methods are preferable for the removal of hydrated chromium oxide formed on the metallic chromium layer. One is the method wherein the chromium plated steel base is cathodically treated in an acid solution such as sulfuric acid and hydrochloric acid having a pH of 0.5 to 2.0, before nickel-zinc alloy plating. The other is the method wherein nickel-zinc alloy plating is carried out at the same time with the removal of hydrated chromium oxide formed on the metallic chromium layer by using a nickel-zinc alloy plating electrolyte having a low pH

of 0.5 to 2.0 which has a low current efficiency for the deposition of nickel-zinc alloy.

The conditions for the removal of hydrated chromium oxide by the former method are as follows:

5 Electrolyte: An acid solution containing at least one acid selected from the group consisting of sulfuric acid, hydrochloric acid, hydro-fluoric acid, fluoboric acid and fluosilicic acid having a pH of 0.5 to 2.0

10 Temperature of the electrolyte: 30°-70° C.

Cathodic current density: 2-50 A/dm<sup>2</sup>

Treating time: 0.5-5.0 seconds

15 Although the main component in the electrolyte is sulfuric acid and/or hydrochloric acid, if the pH of the electrolyte is kept between 0.5 to 2.0, various ions, which are not deposited on the surface of the chromium plated steel base or do not oxidize the surface of the chromium plated steel base, can be contained in the electrolyte. It is not necessary that the temperature of the electrolyte be strictly controlled if it is kept between 30° to 70° C.

20 If the temperature of the electrolyte is above 70° C., the evaporation of water is increased. At below 30° C. a cathodic treatment for a long time is required for a sufficient removal of hydrated chromium oxide.

25 At below 2 A/dm<sup>2</sup> of current density, hydrated chromium oxide is not sufficiently removed, even if the chromium plated steel base is cathodically treated for a long time. An upper limit of current density is limited to 50 A/dm<sup>2</sup> because the effect of the present treatment is not increased in a current density above 50 A/dm<sup>2</sup>.

30 If the treating time is below 0.5 seconds, hydrated chromium oxide is not sufficiently removed from the metallic chromium layer, even if the higher current density is applied. The treating time above 5.0 seconds is not suitable in the high speed production of TFS-CNZT according to the present invention.

35 The conditions for the latter method wherein nickel-zinc alloy plating is carried out at the same time with the removal of hydrated chromium oxide formed on the metallic chromium layer is as follows:

Concentration of nickel ion: 15-80 g/l

Concentration of zinc ion: 0.5-16 g/l

Concentration ratio of zinc ion to nickel ion: 0.03-0.2  
40 pH of the electrolyte: 0.5-2.0

Temperature of the electrolyte: 30°-70° C., more preferably 30°-50° C.

45 Cathodic current density: 2-50 A/dm<sup>2</sup>, more preferably 2-30 A/dm<sup>2</sup>

50 In this method, it is very important that the concentration ratio of zinc ion to nickel ion is kept within the range described above in order to obtain nickel-zinc alloy containing 10 to 90 weight percent of zinc on the chromium plated steel base. If the concentration ratio of zinc ion to nickel ion is below 0.03, nickel-zinc alloy having above 10 weight percent of zinc is not obtained.

55 The zinc content in the plated nickel-zinc alloy increases with an increase of the concentration ratio of zinc ion to nickel ion. At above 0.2 of the concentration ratio of zinc ion to nickel ion, nickel-zinc alloy containing a small amount of nickel is obtained.

60 It is not suitable in the present invention that the concentration of nickel ion is below 15 g/l because it is difficult to control exactly the concentration of zinc ion at below 0.5 g/l and the zinc content in the plated nickel-zinc alloy may change by the presence of a small amount of ions such as chromium ion and iron ion

which are built up in the electrolyte by a dissolution of hydrated chromium oxide and the steel base.

The concentration of nickel ion is limited to 80 g/l from the standpoint of resource conservation, although the effect of the present plating is not decreased at a concentration above 80 g/l, if the concentration ratio of zinc ion to nickel ion is kept within the range of 0.03 to 0.2. The upper limit in the concentration of zinc ion is naturally decided to 16 g/l from the upper limit of the concentration of nickel ion in order to obtain nickel-zinc alloy having 10 to 90 weight percent of zinc.

Nickel ion is mainly supplied by the addition of nickel sulfate, nickel chloride and nickel sulfamate or the dissolution of a soluble nickel anode. And zinc ion is also mainly supplied by the addition of zinc sulfate, zinc chloride and zinc hydroxide or the dissolution of a soluble zinc anode. Additives such as sodium sulfate, ammonium sulfate, ammonium chloride, boric acid and organic additives which are used in a known nickel plating electrolyte or a known zinc plating electrolyte can be used for the improvement of the uniformity of the plated nickel-zinc alloy and the conductivity of the electrolyte, if the concentration ratio of zinc ion to nickel and the pH of the nickel-zinc alloy plating electrolyte are kept within the range described above, respectively.

The pH of the electrolyte is very important for nickel-zinc alloy plating on the chromium plated steel base with the removal of hydrated chromium oxide formed on the metallic chromium layer in the present invention. The pH range of the electrolyte should be from 0.5 to 2.0, preferably 0.5 to 1.5.

At a low pH such as 0.5 to 2.0, the surface of the chromium plated steel base is uniformly activated because hydrated chromium oxide formed during chromium plating is easily removed from the chromium plated steel base by the evolution of a large amount of hydrogen and the dissolving action by acid.

Therefore a uniform nickel-zinc alloy layer is formed on the metallic chromium layer. A pH of below 0.5 is not desirable in the present invention, because a part of metallic chromium may be dissolved. And the pH of above 2.0 is also not desirable in high speed production of TFS-CNZT according to the present invention because the uniform nickel-zinc alloy layer is not formed on the metallic chromium layer by the insufficient dissolution of hydrated chromium oxide for a short time.

Furthermore, it is difficult to produce TFS-CNZT stably because the pH of the electrolyte changes considerably by a slight change in the concentration of metal ion and acid.

The pH of the electrolyte is mainly controlled by the addition of sulfuric acid, hydrochloric acid, hydrofluoric acid, fluoroboric acid and fluosilicic acid. Various ions, which do not give bad effects for nickel-zinc alloy plating and the dissolution of hydrated chromium oxide, may be contained in the electrolyte if the pH of the electrolyte is kept in the range of from 0.5 to 2.0.

It is suitable in the present invention that the range of the cathodic current density is 2 to 50 A/dm<sup>2</sup>, more preferably 2 to 30 A/dm<sup>2</sup>. If the current density is below 2 A/dm<sup>2</sup>, the current efficiency for nickel-zinc alloy plating by this electrolyte becomes so low that a long time is necessary for the deposition of the required amount of nickel and zinc. If the current density is above 50 A/dm<sup>2</sup>, it is difficult to deposit nickel-zinc alloy having 20 to 90 weight percent of zinc because of the formation of nickel hydroxide.

The optimum range for the temperature of the electrolyte is from 30° to 70° C., more preferably 30° to 50° C. At below 30° C., hydrated chromium oxide is not dissolved sufficiently, so that the uniform nickel-zinc alloy layer is not plated on the chromium plated steel base. At above 70° C., a part of metallic chromium is dissolved along with hydrated oxide.

Both cathodic treatment in an acidic solution having a pH of 0.5 to 2.0 and nickel-zinc alloy plating with the removal of hydrated chromium oxide formed during chromium plating described above are also applied for the removal of hydrated chromium oxide in the case of drying after chromium plating and water rinsing under the same conditions described above.

In the case of nickel-zinc alloy plating after the removal of hydrated chromium oxide by a cathodic treatment of the chromium plated steel base in an acidic solution such as sulfuric acid and hydrochloric acid, nickel-zinc alloy plating is also carried out by using the same electrolyte and the same plating conditions described above. In this case, nickel-zinc alloy plating electrolyte wherein zinc sulfate, zinc chloride and/or zinc hydroxide is added to a known nickel plating electrolyte such as Watts bath or nickel sulfamate bath having a high pH of 3 to 5.5 can be also used for nickel-zinc alloy plating on the chromium plated steel base, because hydrated chromium oxide formed during chromium plating is sufficiently removed by a cathodic treatment of the chromium plated steel base in an acidic solution such as sulfuric acid and hydrochloric acid.

Therefore, the following conditions for nickel-zinc alloy plating is used in this case:

Concentration of nickel ion: 15-80 g/l

Concentration of zinc ion: 0.5-16 g/l

Concentration ratio of zinc ion to nickel ion: 0.03-0.2  
pH of the electrolyte: 0.5-5.5

Temperature of the electrolyte: 30°-70° C.

Cathodic current density: 2-50 A/dm<sup>2</sup>

In the present invention, two types of the electrolytes are used for the formation of hydrated chromium oxide as a top layer of the TFS-CNZT. The first type of the electrolyte, which is used for the post-treatment of electrotinplate, consists of an acidic chromate electrolyte without addition of additives such as fluorine compounds and sulfur compounds. The second type of the electrolyte, which is used for the production of TFS-CT having a lower layer of metallic chromium and an upper layer of hydrated chromium oxide, consists of chromic acid electrolyte with additives such as fluorine compounds and sulfur compounds.

It is suitable to employ the following conditions for the formation of hydrated chromium oxide of 2 to 18 mg/m<sup>2</sup> as chromium by using the first type of the electrolyte:

Concentration of hexavalent chromium ion: 5-30 g/l

Temperature of the electrolyte: 30°-70° C.

Cathodic current density: 1-20 A/dm<sup>2</sup>

Quantity of electricity: 1-40 coulombs/dm<sup>2</sup>

If the concentration of hexavalent chromium ion is below 5 g/l, waste of electric power results from the higher electric resistance of the electrolyte. The concentrations of hexavalent chromium ion is limited to 30 g/l from the viewpoint of conserving resources, although the effect of the present treatment is not decreased in a concentration above 30 g/l.

It is an essential condition that the electrolyte should be acidified. In the case of an alkaline electrolyte, the efficiency for the formation of hydrated chromium

oxide is so low that a long time is necessary for the formation of a suitable amount of hydrated chromium oxide. Therefore, the electrolyte containing only a chromate of an alkali metal or ammonium is not used in the present invention.

In the above case the alkaline electrolyte should be acidified by the addition of chromic acid. It is also possible to add a hydroxide of an alkali metal or ammonium to chromic acid electrolyte within an acid range.

Therefore at least one chromate selected from the group consisting of chromic acid, a chromate and dichromate of an alkali metal, ammonium chromate and ammonium dichromate is used for the first type of the electrolyte within an acid range in the present invention. It is not necessary that the temperature of the electrolyte be strictly controlled if it is kept between 30° to 70° C.

If the temperature of the electrolyte above 70° C., the evaporation of water is increased.

Under a current density below 1 A/dm<sup>2</sup>, a long time is necessary for the formation of a suitable amount of hydrated chromium oxide. Under a current density above 20 A/dm<sup>2</sup>, the control in the amount of the formed hydrated chromium oxide may be difficult because a large amount of hydrated chromium oxide is formed by a cathodic treatment for a short time.

If the quantity of electricity is below 1 coulomb/dm<sup>2</sup>, it is difficult to form a suitable amount of hydrated chromium oxide.

At above 40 coulombs/dm<sup>2</sup> of the quantity of electricity, the weldability of the TFS-CN<sub>2</sub>T according to the present invention becomes poor because of the formation of thicker hydrated chromium oxide.

It is desirable, to employ the following conditions for the formation of hydrated chromium oxide by using the second type of the electrolyte:

Concentration chromic acid: 10-50 g/l

Weight percent of additives to chromic acid: 0.2-1.0  
Additives: Sulfur compound and/or fluorine compound

Temperature of the electrolyte: 30°-60° C.

Cathodic current density: 1-10 A/dm<sup>2</sup>

In the conditions described above, weight ratio of additives to chromic acid and current density are very important in the present treatment, because at a higher weight ratio of additives to chromic acid and higher current density, metallic chromium which gives a bad effect to the weldability of TFS-CN<sub>2</sub>T, is deposited on the nickel-zinc alloy plated steel base. Therefore, the weight ratio of additives to chromic acid is limited to 1.0 and a cathodic current density is limited to 10 A/dm<sup>2</sup>. However, if the weight ratio of additives to chromic acid is below 0.2, the weldability becomes poor because thick hydrated chromium oxide is formed. Under a current density below 1 A/dm<sup>2</sup>, a long time is necessary for the formation of a suitable amount of hydrated chromium oxide. Furthermore, the ranges in the concentration of chromic acid, the quantity of electricity and the temperature of the electrolyte are limited as in the first type of the electrolyte by the same reason.

Additives are also selected from the same group as in chromium plating electrolytes.

In the treatment using the second type of electrolyte, it is very important to select the conditions wherein metallic chromium is not deposited on the nickel-zinc alloy plated surface.

However, under some conditions wherein metallic chromium is deposited, the maximum amount of metallic chromium deposited on the nickel-zinc alloy plated

surface should be limited to 10 mg/m<sup>2</sup>, although the amount of the deposited metallic chromium should be ideally zero.

The present invention is illustrated by the following Examples.

In Example 1 and Example 2, a cold rolled steel sheet having a thickness of 0.22 mm was treated by the following process after electrolytically degreasing in a solution of 70 g/l of sodium hydroxide, water rinsing, pickling in solution of 100 g/l of sulfuric acid and water rinsing.

Chromium plating → water rinsing → nickel-zinc alloy plating → water rinsing → chromate treatment → water rinsing → drying.

In Example 3 and 4, the same kind of steel sheet pre-treated as in Example 1 and Example 2 was treated by the following process.

Chromium plating → water rinsing → the removal of hydrated chromium oxide formed during chromium plating by a cathodic treatment in an acidic solution → water rinsing → nickel-zinc alloy plating → water rinsing → chromate treatment → water rinsing → drying.

In each Example, the conditions are shown in detail.

## EXAMPLE 1

### Conditions for chromium plating

#### Composition of electrolyte

CrO<sub>3</sub>: 120 g/l

HBF<sub>4</sub>: 0.8 g/l

H<sub>2</sub>SO<sub>4</sub>: 0.5 g/l

Temperature of electrolyte: 60° C.

Cathodic current density: 50 A/dm<sup>2</sup>

### Conditions for nickel-zinc alloy plating

#### Composition of electrolyte

Ni(NH<sub>2</sub>SO<sub>3</sub>)<sub>2</sub>.4H<sub>2</sub>O: 20 g/l as Ni<sup>2+</sup>

ZnSO<sub>4</sub>.7H<sub>2</sub>O: 0.7 g/l as Zn<sup>2+</sup>

H<sub>3</sub>BO<sub>3</sub>: 40 g/l

Ratio of Zn<sup>2+</sup> to Ni<sup>2+</sup>: 0.035

pH (by addition of H<sub>2</sub>SO<sub>4</sub>): 0.6

Temperature of electrolyte: 60° C.

Cathodic current density: 50 A/dm<sup>2</sup>

### Conditions for chromate treatment

#### Composition of electrolyte

CrO<sub>3</sub>: 30 g/l

Na<sub>2</sub>SiF<sub>6</sub>: 0.1 g/l

Temperature of electrolyte: 60° C.

Cathodic current density: 5 A/dm<sup>2</sup>

## EXAMPLE 2

### Conditions for chromium plating

#### Composition of electrolyte

CrO<sub>3</sub>: 100 g/l

NaF: 5 g/l

Temperature of electrolyte: 55° C.

Cathodic current density: 30 A/dm<sup>2</sup>

### Conditions for nickel-zinc alloy plating

#### Composition of electrolyte

NiSO<sub>4</sub>.6H<sub>2</sub>O: 75 g/l as Ni<sup>2+</sup>

ZnCl<sub>2</sub>: 15 g/l as Zn<sup>2+</sup>

Ratio of Zn<sup>2+</sup> to Ni<sup>2+</sup>: 0.20

pH (by addition of HCl): 2.0

Temperature of electrolyte: 30° C.

Cathodic current density: 30 A/dm<sup>2</sup>

- Conditions for chromate treatment  
 Composition of electrolyte  
 CrO<sub>3</sub>: 30 g/l  
 H<sub>2</sub>SO<sub>4</sub>: 0.1 g/l  
 Temperature of electrolyte: 60° C.  
 Cathodic current density: 10 A/dm<sup>2</sup>

## EXAMPLE 3

- Conditions for chromium plating  
 Composition of electrolyte  
 CrO<sub>3</sub>: 200 g/l  
 NaF: 6 g/l  
 Na<sub>2</sub>SiF<sub>6</sub>: 2 g/l  
 Temperature of electrolyte: 50° C.  
 Cathodic current density: 40 A/dm<sup>2</sup>
- Conditions for the removal of hydrated chromium oxide  
 Composition of electrolyte  
 H<sub>2</sub>SO<sub>4</sub>: pH 0.5  
 Temperature of electrolyte: 60° C.  
 Cathodic current density: 20 A/dm<sup>2</sup>  
 Treating time: 0.5 seconds
- Conditions for nickel-zinc alloy plating  
 Composition of electrolyte  
 NiSO<sub>4</sub>·6H<sub>2</sub>O: 80 g/l as Ni<sup>2+</sup>  
 ZnSO<sub>4</sub>·7H<sub>2</sub>O: 6 g/l as Zn<sup>2+</sup>  
 H<sub>3</sub>BO<sub>3</sub>: 30 g/l  
 Ratio of Zn<sup>2+</sup> to Ni<sup>2+</sup>: 0.075  
 pH (no addition of acid): 4.8  
 Temperature of electrolyte: 40° C.  
 Cathodic current density: 2 A/dm<sup>2</sup>

## Conditions for chromate treatment

- Composition of electrolyte  
 CrO<sub>3</sub>: 50 g/l  
 H<sub>2</sub>SO<sub>4</sub>: 0.1 g/l  
 Temperature of electrolyte: 50° C.  
 Cathodic current density: 5 A/dm<sup>2</sup>

## EXAMPLE 4

- Conditions for chromium plating  
 Composition of electrolyte  
 CrO<sub>3</sub>: 80 g/l  
 NaF: 4 g/l  
 Temperature of electrolyte: 50° C.  
 Cathodic current density: 30 A/dm<sup>2</sup>
- Conditions for the removal of hydrated chromium oxide  
 Composition of electrolyte  
 HCl: pH 2.0  
 Temperature of electrolyte: 40° C.  
 Cathodic current density: 5 A/dm<sup>2</sup>  
 Treating time: 3 seconds
- Conditions for nickel-zinc alloy plating  
 NiSO<sub>4</sub>·6H<sub>2</sub>O: 20 g/l as Ni<sup>2+</sup>  
 ZnSO<sub>4</sub>·7H<sub>2</sub>O: 2 g/l as Zn<sup>2+</sup>  
 H<sub>3</sub>BO<sub>3</sub>: 40 g/l  
 Ratio of Zn<sup>2+</sup> to Ni<sup>2+</sup>: 0.1  
 pH (no addition of acid): 5.4  
 Temperature of electrolyte: 60° C.  
 Cathodic current density: 5 A/dm<sup>2</sup>

- Conditions for chromate treatment  
 Composition of electrolyte

- Na<sub>2</sub>Cr<sub>2</sub>O<sub>7</sub>·2H<sub>2</sub>O: 30 g/l  
 Temperature of electrolyte: 50° C.  
 Cathodic current density: 2 A/dm<sup>2</sup>

## COMPARATIVE EXAMPLE 1

The same kind of steel sheet pretreated as in Example 1 was treated under the following conditions and was then rinsed with water and dried.

- 10 Conditions of electrolytic chromic acid treatment  
 Composition of electrolyte  
 CrO<sub>3</sub>: 80 g/l  
 HBF<sub>4</sub>: 0.5 g/l  
 H<sub>2</sub>SO<sub>4</sub>: 0.5 g/l  
 Temperature of electrolyte: 45° C.  
 Cathodic current density: 20 A/dm<sup>2</sup>

## COMPARATIVE EXAMPLE 2

The same kind of steel sheet pretreated as in Example 1 was plated with nickel-zinc alloy under the following conditions.

- Conditions for nickel-zinc alloy plating  
 Composition of electrolyte  
 NiSO<sub>4</sub>·6H<sub>2</sub>O: 20 g/l as Ni<sup>2+</sup>  
 ZnSO<sub>4</sub>·7H<sub>2</sub>O: 3 g/l as Zn<sup>2+</sup>  
 H<sub>3</sub>BO<sub>3</sub>: 40 g/l  
 Ratio of Zn<sup>2+</sup> to Ni<sup>2+</sup>: 0.15  
 pH (no addition of acid): 5.4  
 Temperature of electrolyte: 55° C.  
 Cathodic current density: 10 A/dm<sup>2</sup>  
 After rinsing with water, the nickel-zinc alloy plated steel sheet was treated under the following conditions and was then rinsed with water and dried.

## Conditions for chromate treatment

- Composition of electrolyte  
 Na<sub>2</sub>Cr<sub>2</sub>O<sub>7</sub>·2H<sub>2</sub>O: 30 g/l  
 Temperature of electrolyte: 40° C.  
 Cathodic current density: 10 A/dm<sup>2</sup>

## COMPARATIVE EXAMPLE 3

The same kind of steel sheet pretreated as in Example 1 was plated with chromium by using an aqueous electrolyte containing 100 g/l of CrO<sub>3</sub> and 5 g/l of NaF under a current density of 30 A/dm<sup>2</sup> at temperature of 55° C. After rinsing with water, the chromium plated steel sheet with hydrated chromium oxide of about 3 mg/m<sup>2</sup> as chromium was plated with nickel under the following conditions.

- Conditions for nickel plating  
 Composition of electrolyte  
 NiSO<sub>4</sub>·6H<sub>2</sub>O: 55 g/l as Ni<sup>2+</sup>  
 H<sub>3</sub>BO<sub>3</sub>: 30 g/l  
 pH (by addition of H<sub>2</sub>SO<sub>4</sub>): 0.5  
 Temperature of electrolyte: 40° C.  
 Cathodic current density: 5 A/dm<sup>2</sup>  
 After rinsing with water, the chromium and nickel-zinc alloy plated steel sheet was treated by using 30 g/l of Na<sub>2</sub>Cr<sub>2</sub>O<sub>7</sub>·2H<sub>2</sub>O under a current density of 5 A/dm<sup>2</sup> at a temperature of 40° C. and was then rinsed with water and dried.

The weldability, lacquer adhesion and corrosion resistance of thus treated steel sheet in the above described Examples and Comparative examples were evaluated by the following testing methods after the measurements of the amounts of metallic chromium,

nickel, zinc and chromium in hydrated chromium oxide by the fluorescent X-ray method.

The results of tests are shown in the attached Table.

(1) Weldability

The weldability is usually evaluated by an available range of secondary current in welding as shown in the report by N. T. Williams (Metal Construction, April 1977, page 157-160), that is to say, the wider the secondary current range in welding, the better the weldability. The upper limit in the available secondary current range corresponds to the welding conditions in which some defect such as splashing is found and the lower limit corresponds to the welding conditions in which the breakage occurs in the welded part by tearing tests.

However, in order to obtain data wherein the available range of secondary current in welding is decided in each sample, a large number of samples are necessary.

Therefore, the weldability was evaluated by an electric contact resistance according to the following methods, because an electric contact resistance has an apparent correlation with an available range of secondary current in welding as shown in the report by T. Fujimura (Journal of The Iron and Steel Institute of Japan, vol. 69, No. 13, September 1983, page 181), that is, the lower the electric contact resistance, the wider the secondary current range in welding. Accordingly, if the electric contact resistance is lower, the weldability

5

10

15

20

25

The coated sample was cut into a circular blank having a diameter of 80 mm by a punch press, and the blank was deeply drawn to form a cup.

The lacquer film in the side wall of a cup was peeled off by an adhesive tape. The adhesion of the lacquer film was divided into 5 ranks, namely, 5 was excellent, 4 was good, 3 was fair, 2 was poor and 1 was bad.

(3) Corrosion resistance after lacquer coating

The sample was aked at 210° C. for 12 minutes after coating with 60 mg/dm<sup>2</sup> of an epoxy-phenolic type of lacquer. The coated sample was immersed into the solution containing 1.5% of citric acid and 1.5% of sodium chloride for 7 days at 50° C., after the surface of the coated sample was crosshatched by a razor.

The corrosion in the scratched part of the coated sample was divided into 5 ranks, namely, 5 was excellent, 4 was good, 3 was fair, 2 was poor and 1 was bad.

(4) Sulfide stain resistance after lacquer coating

The sample was baked at 210° C. for 12 minutes after coating with 60 mg/dm<sup>2</sup> of an epoxy-phenolic type of lacquer. The coated sample was formed into a can end by a press. The lacquered can end was treated in a retort at 130° C. for 3 hours after the immersion into a solution containing tuna meat with oil which had been deaerated by boiling. The sulfide stain resistance of the lacquered can end was divided into 5 ranks by a degree of blackening, namely, 5 was excellent (no change), 4 was good, 3 was fair, 2 was poor and 1 was bad.

TABLE

|                                                                                 | Ex. 1   | Ex. 2    | Ex. 3    | Ex. 4     | Comp. Ex. 1 | Comp. Ex. 2 | Comp. Ex. 3 |
|---------------------------------------------------------------------------------|---------|----------|----------|-----------|-------------|-------------|-------------|
| * <sup>1</sup> Process                                                          | A       | A        | B        | B         | —           | —           | A           |
| * <sup>2</sup> Amount of Cr <sup>o</sup> (mg/m <sup>2</sup> )<br>(Bottom layer) | 80      | 35       | 122      | 285       | 118         | —           | 124         |
| Amount of Ni & Zn (mg/m <sup>2</sup> )<br>(Middle layer)                        | Ni<br>3 | Ni<br>17 | Ni<br>34 | Ni<br>53  | —           | Ni<br>18    | Ni<br>48    |
|                                                                                 | Zn<br>5 | Zn<br>18 | Zn<br>11 | Zn<br>196 | —           | Zn<br>17    | Zn<br>0     |
| * <sup>2</sup> Amount of Cr <sup>ox</sup> (mg/m <sup>2</sup> )<br>(Top layer)   | 10      | 4        | 8        | 15        | 15          | 11          | 7           |
| Electric contact<br>resistance (mΩ)                                             | 16      | 8        | 6        | 10        | 328         | 108         | 18          |
| Lacquer adhesion                                                                | 5       | 5        | 5        | 5         | 5           | 4           | 5           |
| Corrosion resistance<br>after lacquering                                        | 5       | 5        | 5        | 4         | 5           | 3           | 5           |
| Sulfide stain<br>resistance                                                     | 5       | 5        | 5        | 5         | 5           | 3           | 3           |

## Remarks

\*<sup>1</sup>Process A Chromium plating—Water rinsing—Nickel-zinc alloy plating—Water rinsing—Chromate treatment—Water rinsing—Drying

Process B Chromium plating—Water rinsing—Cathodic treatment in acid solution—Water rinsing—Nickel-zinc alloy plating—Water rinsing—Chromate treatment—Water rinsing—Drying

\*<sup>2</sup>Cr<sup>o</sup> shows metallic chromium and Cr<sup>ox</sup> shows Cr in hydrated chromium oxide.

\*<sup>3</sup>In Comparative example 3, nickel plating was carried out instead of nickel-zinc alloy plating.

## We claim:

1. A tin free steel having three layers consisting of a bottom layer of metallic chromium, a middle layer of nickel-zinc alloy and a top layer of hydrated chromium oxide on a steel base.

2. The tin free steel according to claim 1, wherein the amount of metallic chromium in said bottom layer is from 30 to 300 mg/m<sup>2</sup>, the amount of nickel-zinc alloy in said middle layer is from 5 to 300 mg/m<sup>2</sup> and the amount of hydrated chromium oxide in said top layer is from 2 to 18 mg/m<sup>2</sup> as chromium.

3. The tin free steel according to claim 2, wherein the amount of metallic chromium in said bottom layer is from 70 to 150 mg/m<sup>2</sup>, the amount of nickel-zinc alloy in said middle layer is from 5 to 50 mg/m<sup>2</sup> and the amount of hydrated chromium oxide in said top layer is from 4 to 12 mg/m<sup>2</sup> as chromium.

is better.

At first, the sample treated on both sides was cut to a size of 20 mm×100 mm after baking at 210° C. for 20 minutes.

The electric contact resistance of the sample was calculated from the change of voltage between a pair of copper disk electrodes (diameter: 65 mm, thickness 2 mm) wherein 5 amperes of direct current were supplied and 50 kg of load was added, when two sample pieces were inserted into between a pair of the copper disk electrodes rotating at 5 m/min.

(2) Lacquer adhesion

The sample was baked at 210° C. for 12 minutes after coating with 60 mg/dm<sup>2</sup> of an epoxy-phenolic type of lacquer.

55

60

65

4. The tin free steel according to claim 1, wherein nickel-zinc alloy in said middle layer contains 10 to 90 weight percent of zinc.

5. The tin free steel according to claim 4, wherein nickel-zinc alloy in said middle layer contains 10 to 50 weight percent of zinc.

6. A process for continuously preparing a tin free steel as claimed in claim 1, which comprises: (a) chromium plating a steel base to form a layer of metallic chromium and hydrated chromium oxide thereon; (b) nickel-zinc alloy plating the chromium plated steel base using a nickel-zinc alloy plating electrolyte under conditions sufficiently acidic to substantially dissolve said hydrated chromium oxide in said electrolyte; and (c) forming a layer of hydrated chromium oxide on the nickel-zinc alloy plated, chromium plated steel base of step (b).

7. The process according to claim 6, wherein said nickel-zinc alloy plating of the chromium plated steel base with the removal of hydrated chromium oxide formed on the chromium plated steel base is carried out at a temperature of 30° to 70° C. and under a cathodic current density of 2 to 50 A/dm<sup>2</sup> by using a nickel-zinc alloy plating electrolyte having 15 to 80 g/l of nickel ion, 0.5 to 16 g/l of zinc ion, 0.03 to 0.2 of concentration ratio of zinc ion to nickel ion and a pH of 0.5 to 2.0.

8. The process for continuously preparing a tin free steel as claimed in claim 1, which comprises: (a) chromium plating a steel base to form a layer of metallic chromium and hydrated chromium oxide thereon; (b) removing the hydrated chromium oxide formed on the chromium plated steel base by a cathodic treatment in an acidic solution; (c) nickel-zinc alloy plating the chromium plated steel base; and (d) forming a layer of hydrated chromium oxide on the nickel-zinc alloy plated, chromium plated steel base of step (c).

9. The process according to claim 8, wherein said removal of hydrated chromium oxide formed on the chromium plated steel base is carried out at a temperature of 30° to 70° C. and under a cathodic current density of 2 to 50 A/dm<sup>2</sup> and a treating time 0.5 to 5 seconds by using an acidic solution containing at least one acid selected from the group consisting of sulfuric acid, hydrochloric acid, hydrofluoric acid, fluoboric acid and fluosilicic acid and having a pH of 0.5 to 2.0.

10. The process according to claim 8, wherein said nickel-zinc alloy plating on the chromium plated steel base is carried out at a temperature of 30° to 70° C. and under a cathodic current density of 2 to 50 A/dm<sup>2</sup> by using a nickel-zinc alloy plating electrolyte having 15 to 80 g/l of nickel ion, 0.5 to 16 g/l of zinc ion, 0.03 to 0.2 of concentration ratio of zinc ion to nickel ion and a pH of 0.5 to 5.5.

11. The process according to claim 6 or 8, wherein said chromium plating of the steel base is carried out at a temperature of 30° to 60° C. and under a cathodic current density of 10 to 100 A/dm<sup>2</sup> in an electrolyte containing 30 to 300 g/l of chromic acid and at least one additive selected from the group consisting of a fluorine compound and a sulfur compound wherein the amount

of said additive being 1 to 5 weight percent of chromic acid.

12. The process according to claim 11, wherein said fluorine compound is at least one compound selected from the group consisting of hydrofluoric acid, fluoboric acid, fluosilicic acid, ammonium bifluoride, an alkali metal bifluoride, ammonium fluoride, an alkali metal fluoride, ammonium fluoborate, an alkali metal fluoborate, ammonium fluosilicate, an alkali metal fluosilicate and aluminum fluoride.

13. The process according to claim 11, wherein said sulfur compound is at least one compound selected from the group consisting of sulfuric acid, ammonium sulfate, an alkali metal sulfate, phenolsulfonic acid, ammonium phenolsulfonate, an alkali metal phenolsulfonate, phenoldisulfonic acid, ammonium phenoldisulfonate, an alkali metal phenoldisulfonate, ammonium sulfite, an alkali metal sulfite, ammonium thiosulfate, an alkali thiosulfate, aluminum sulfate and chromium sulfate.

14. The process according to claim 6 or 8, wherein said hydrated chromium oxide is formed on the nickel-zinc alloy plated steel base by a cathodic treatment in an acidic electrolyte containing at least one compound selected from the group consisting of chromic acid, a chromate and a dichromate of an alkali metal, ammonium chromate and ammonium dichromate.

15. The process according to claim 14, wherein said cathodic treatment is carried out at a temperature of 30° to 70° C. and under a cathodic current density of 1 to 20 A/dm<sup>2</sup>, a quantity of electricity of 1 to 40 coulombs/dm<sup>2</sup> in an acidic electrolyte containing 5 to 30 g/l of hexavalent chromium ion.

16. The process according to claim 6 or 8, wherein said hydrated chromium oxide is formed on the nickel-zinc alloy plated steel base by a cathodic treatment in an acidic electrolyte containing 10 to 50 g/l of chromic acid and at least one additive selected from the group consisting of a fluorine compound and a sulfur compound wherein the amount of said additive being 0.2 to 1.0 weight percent of chromic acid.

17. The process according to claim 16, wherein said cathodic treatment is carried out at a temperature of 30° to 60° C. and under a cathodic current density of 1 to 10 A/dm<sup>2</sup>, a quantity of electricity of 1 to 20 coulombs/dm<sup>2</sup>.

18. The process according to claim 16, wherein said fluorine compound is at least one compound selected from the group consisting of hydrofluoric acid, fluoboric acid, fluosilicic acid, ammonium bifluoride, an alkali metal bifluoride, ammonium fluoride, an alkali metal fluoride, ammonium fluoborate, an alkali metal fluoborate, ammonium fluosilicate, an alkali metal fluosilicate and aluminum fluoride.

19. The process according to claim 16, wherein said sulfur compound is at least one compound selected from the group consisting of sulfuric acid, ammonium sulfate, an alkali metal sulfate, phenolsulfonic acid, ammonium phenolsulfonate, an alkali metal phenolsulfonate, phenoldisulfonic acid, ammonium phenoldisulfonate, an alkali metal phenoldisulfonate, ammonium sulfite, an alkali metal sulfite, ammonium thiosulfate, an alkali metal thiosulfate, and chromium sulfate.

\* \* \* \* \*